# EUROPEAN PATENT SPECIFICATION

(11) **EP 2 838 096 B1**
(45) Date of publication and mention of the grant of the patent: **19.07.2017**
(21) Application number: 14179785.2
(22) Date of filing: 05.08.2014
(51) Int. Cl.: H01H 1/0233, H01H 1/025

(54) **Electrical contact system**
Elektrisches Kontaktsystem
Système de contact électrique

(30) Priority: 16.08.2013 IN CH36372013
(43) Date of publication of application: 18.02.2015
(73) Proprietor: General Electric Company, Schenectady, NY 12345 (US)
(72) Inventor: Karkada, Nagaveni, 560066 Karnataka (IN); Ramachandran, Gopi Chandran, 560066 Karnataka (IN); Asokan, Thangavelu, 560037 Karnataka (IN)
(74) Representative: Fischer, Jens Peter

(56) References cited:
- US-A- 1 342 801
- US-A- 5 139 890
- US-A1- 2008 199 716

## Description

### BACKGROUND

The present invention relates generally to a contact arm assembly having an electrical contact in an electrical circuit breaker.

Contacts and contact arm assemblies are well known in the art of circuit breakers. Contact arm assemblies having electrical contacts for making and breaking an electrical current are not only employed in electrical circuit breakers, but also in other electrical devices, such as rotary double break circuit breakers, contactors, relays, switches, and disconnects. The applications that these electrical devices are used in are vast and include, but are not limited to, the utility, industrial, commercial, residential, and automotive industries.

The primary function of a contact arm assembly is to provide a carrier for an electrical contact that is capable of being actuated in order to separate the contact from a second contact and contact arm arrangement, thereby enabling the making and breaking of an electrical current in an electric circuit. Electrical contacts suitable for the noted applications typically include silver.

The contact is generally bonded to the contact arm, which is typically, but not necessarily, a copper alloy, in such a manner that the assembly tolerates the thermal, electrical and mechanical stresses and will not disassemble during operation of the host device. Predominantly the contact failure occurs due to wear and tear. Factors that normally affect contact and trigger wear and tear are configuration or geometry of contact (different layer/thickness), materials choice, and processing (brazing/ welding) that creates voids at the interface. Hence there is a need for improved assembly of the contacts with high interfacial quality. The system and method presented herein are directed towards addressing this need.

US 5,139,890 discloses silver-coated electrical components.

US 1,342,801 discloses a contact tip (arcing terminal) comprising an arcing surface (B); a base surface (A); and a graded structure between the arcing surface and the base surface, wherein the graded structure comprises a first region; a second region; and an intermediate region (between A and B) disposed between the first region and the second region; the first region contains silver; the intermediate region contains silver; and the concentration of silver in the intermediate region is less than the concentration of silver in the first region.

### BRIEF DESCRIPTION

In one embodiment, a system is presented. The system includes a contact tip that includes an arcing surface, a base surface, and a graded structure between the arcing surface and the base surface. The graded structure includes a first region comprising a first surface proximate to the arcing surface, a second region comprising a second surface proximate to the base surface, and an intermediate region disposed between the first region and the second region. Further, a concentration of silver in the graded structure decreases from the first surface to the second surface.

In one embodiment, a method of forming a contact tip is presented. The method includes preparing starting materials for a first region, an intermediate region, and a second region of the contact tip. The starting materials of the first, intermediate, and second regions are sequentially added to a container to form a graded blend of starting materials. The graded blend of starting materials are compacted and heat-treated to form a contact tip having a graded structure. The graded structure has a concentration of silver decreasing from the first region to the second region.

### BRIEF DESCRIPTION OF DRAWINGS:

FIG. 1 is a schematic diagram of a system including a contact tip, in accordance with one embodiment of the invention;
FIG. 2 is a schematic diagram of a system including one distinctly graded structure, in accordance with one embodiment of the invention;
FIG. 3 is a schematic diagram of a system including one continuously graded structure, in accordance with one embodiment of the invention; and
FIG. 4 is a scanning electron micrograph of a graded structure, in accordance with one embodiment of the invention.

### DETAILED DESCRIPTION

The systems and methods described herein include embodiments that relate to a contact arm assembly having an improved bond between contact and contact arm, thereby enabling the contact arm assembly to withstand thermal, electrical, and mechanical stresses.

In the following specification and the claims that follow, the singular forms "a", "an" and "the" include plural referents unless the context clearly dictates otherwise.

As used herein, the term "adjacent" or "proximate" when used in context of discussion of different compositions or structure of regions or surfaces refers to "immediately next to" and it also refers to the situation wherein other components that are present between the components under discussion do not vary much with regards to the compositions or structure respectively of at least any one of the components.

Referring now to FIG. 1, an exemplary circuit breaker system 10 is shown. The circuit breaker system 10 includes a stationary arm 20 having a fixed contact tip 22 having a fixed base surface 24 and fixed arcing surface 26. The circuit breaker system further includes a moving arm 30 having a movable contact tip 32 having a movable base surface 34 and movable arcing surface 36. The base surfaces 24, 34 of the contact tips 22, 32 are attached to the contact arms 20, 30, and the arcing surfaces 26, 36 are the free surfaces.

During operation, an electric arc occurs between two contact tips 22 and 32 at the arcing surfaces 26, 36 whenever fault current or short circuit happens. The high heat produced by the electric arc may melt both arcing surfaces 26 and 36 and a poor contact between the base 24, 34 and the arcing surfaces 26, 36 may result in transfer of contact materials from one tip to another producing uneven arcing surfaces or carbon slag on the surfaces. The carbon slag produced may adhere to the arcing surfaces 26, 36 and decrease electrical conductivity of the contact subjecting the arcing surfaces 26, 36 to mechanical and electrical degradation. Therefore, it is desired to configure the contact tips 22, 32 with an appropriate hardness, high wear resistance, high temperature stability, and a good bonding between the base surfaces 24, 34 and arcing surfaces 26, 36. Further, the arcing surfaces are desired to be generally inert to oxygen and sulfur reactions.

As alluded above, reliability of contact tips 22, 32 is desired for the increased life of the electrical switch gear. Wear and tear of contacts may be reduced by change in configuration, materials choices, and /or processing. Methods such as extrusion, die compacting, molding are commonly used for manufacturing of arcing surfaces 26, 36.

The arcing surfaces 26, 36 are normally brazed or welded on a copper base 24, 34 in most of the conventional electrical switch gears. Different embodiments of the present invention provide contact tips 22, 32 having graded structure between the base surface and arcing surface, and a new method of fabricating the contact tips 22, 32 without using brazing or welding and thereby eliminating voids in the contact tip 22, 32 structure.

In one embodiment, a circuit breaker system 10 includes a graded structure 40 between the base surface and arcing surface of the fixed contact tip 22 or movable contact tip 32 as shown in FIG. 2. As used herein, the "graded structure between base surface and arcing surface" means that the structure between the base surface and the arcing surface has a gradient from base surface to arcing surface or vice versa. The term "gradient" as used herein means the value of a characteristic parameter of the structure changes with a change in position in the direction from base surface to arcing surface. The characteristic parameter may be composition, density, thickness, reactivity, or microstructure, for example. In one embodiment, the gradient is in the composition of the graded structure.

In one embodiment, both the fixed contact tip 22 and movable contact tip 32 include the graded structure 40. Embodiments described herein use the example of fixed contact tip 22 as having the graded structure 40, while the movable contact tip 32 may or may not have a similar configuration. The graded structure 40 includes a multilayer architecture including a first region 50 proximate to the arcing surface, a second region 60 proximate to the base surface, and an intermediate region 70 disposed between the first region and the second region. The first region 50 includes a first surface 52 facing the arcing surface 26 and the second region 60 includes a second surface 62 facing the base surface 24. The graded structure may optionally have further intermediate regions in between the first and second regions.

In one embodiment, the graded structure 40 includes the first region 50, second region 60, and the intermediate region 70 in distinct, but integrated structure as shown in FIG. 2. In one embodiment, the first region 50, second region 60, and intermediate region 70 are seamless structures integrated to one another according to their layered positions as shown in FIG. 3, but are not distinctly separate in structure from the adjacent regions. The graded structure in this embodiment has a continuously graded structure. The interfaces of continuously graded structures may not be apparent at the macroscopic level, but may have interfaces of layers that can be identified at microscopic scale.

The distinct or continuous multilayer architecture described herein is configured to be free of defects or voids and designed to be robust towards wear. This multilayer structure has superior mechanical strength, heat dissipation, and electrical performance over the current design of contacts. The graded architecture promotes reliable contact configuration, and may be formed by additive manufacturing, thereby eliminating brazing or joining of metals.

Silver is considered to be an excellent contact tip 22 material because of its high thermal and electrical conductivity and considerable inertness to oxygen, nitrogen, and sulfur. However silver has a low melting point, making it prone to fusion and sticking. Further, silver is an expensive material to be used in large quantities. To overcome these challenges, in one embodiment, silver alloys or metal mixtures are used along with silver to increase hardness.

In one embodiment, silver is used as the arcing surface 26, and a concentration of silver in the graded structure 40 decreases from the first surface 52 to the second surface 62. For example, in an example in which graded structure 40 has a distinct multilayered structure, the silver may be decreased from the first surface 52 to the second surface 62 in a stepwise manner. In an embodiment where the layers are in a continuous gradation from the first surface 52 to the second surface 62, the concentration of silver may be continuously decreased from the first surface 52 to the second surface 62. Similarly, a concentration of copper in the graded structure 40 may decrease from the second surface 62 to the first surface 52. In one embodiment, the arcing surface 26 includes substantially 100% silver, and the graded structure 40 may have different regions with decreasing percentage of silver from the first region 50 to the second region 60, and the second surface 62 is substantially free of silver. In one embodiment, the base surface 24 includes substantially 100% copper.

As used herein, "substantially 100%" is used to define the intended 100% composition, but may include any impurities that would not unduly degrade the arcing surface 26 or base surface 24 performance, and further would include any impurities that would have incidentally became incorporated at the surfaces during processing. In one embodiment, the concentration of silver in the arcing surface 26 is greater than about 98% and the concentration of the copper in the base surface 24 is greater than 98%. As used herein the percentages mentioned are weight percentages.

The graded structure 40 used herein may be composed of metals, metal alloys, metal oxides, carbides, or nitrides. In one embodiment, the graded structure 40 includes tungsten, molybdenum, nickel, carbon, or any combinations thereof. The graded structure 40 may include a metal mixture of any of these elements with silver or copper as a part of one or more regions of the graded structure 40. A "metal mixture" as used herein is a mixture of silver or copper with a metal, non-metal, an alloy, or a compound of metal and non-metal. Thus, in one embodiment, the metal mixture may have silver-graphite (alternately silver-carbon) in a mixture form, where the silver and carbon do not generally react with each other to form a compound. In one embodiment, the silver may be in a mixture form with tungsten carbide.

In one embodiment, the metal mixture includes a metal carbide, a silver-tungsten alloy, a silver-nickel alloy, silver-tungsten carbide composite, silver- molybdenum composite, or any combinations of these. In one embodiment, the graded structure 40 has an increasing gradation in the composition of the metal mixture from the surfaces to the center of the graded structure 40. A weight averaged concentration of the metal mixture in the intermediate region 70 of the graded structure 40 may be substantially higher than the concentration of the metal mixture at the first or second regions, when compared to the concentration of silver or copper in the respective regions.

In one embodiment, nickel, carbon, tungsten, molybdenum, and tungsten carbide were studied as individual metal mixtures along with silver, copper, or silver and copper. In one example, the first region 50 includes a silver-nickel metal mixture; the intermediate region 70 includes a silver-copper-nickel metal mixture; and the second region 60 is substantially copper.

In another example, the first region 50 includes a silver-tungsten metal mixture with 35/65 respective weight percentage ratio, the intermediate region 70 includes a silver-copper-tungsten metal mixture with 15/20/65 respective weight percentage ratio, and the second region 60 is substantially copper.

In one more example, the first region 50 includes a silver-graphite metal mixture with 95/5 respective weight percentage ratio, the intermediate region 70 includes a silver-copper-carbide metal mixture with 70/25/5 respective weight percentage ratio, and the second region 60 is substantially copper.

In yet another example, the first region 50 includes a silver-tungsten carbide metal mixture with 35/65 respective weight percentage ratio, the intermediate region 70 includes a copper-tungsten carbide-tungsten metal mixture with 15/20/65 respective weight percentage ratio, and the second region 60 is substantially copper.

In a further example, the first region 50 includes a silver-tungsten carbide metal mixture, the intermediate region 70 includes a silver-copper-tungsten carbide metal mixture, and the second region 60 is substantially copper.

In one more example, the first region 50 includes a silver-tungsten carbide metal mixture, the intermediate region 70 includes a copper-tungsten carbide metal mixture, and the second region 60 is substantially copper.

In one more example, the first region 50 includes a silver-tungsten carbide metal mixture, the intermediate region 70 includes a silver-copper-tungsten carbide metal mixture, and the second region 60 includes a copper-tungsten carbide metal mixture.

In one more example, the first region 50 includes a silver-tungsten carbide metal mixture, the intermediate region 70 includes a copper-tungsten carbide-tungsten metal mixture, and the second region 60 includes a copper-tungsten carbide metal mixture.

FIG. 4 depicts a scanning electron micrograph (SEM) of a graded structure 40. The graded structure includes multiple layers of different concentrations of silver and copper. For example, the first region 50 is of 100% silver, and the second region 60 is of 100% copper. The intermediate regions 70 and 80 vary in the concentration of silver and copper in these layers. For example, layer 70 includes higher concentration of silver than copper and the region 80 includes lower concentration of silver than the amount of copper in that surface.

The contact tip having graded structure 40 may be formed using specific processes that facilitate voidless joining or forming of different regions of the graded structures. For example, methods such as cold pressing, hot pressing, and hot isostatic pressing (HIP) may be used for the formation of graded structure 40.

In one embodiment, powders of different layers are individually blended, arranged in the desired layer configuration and compacted using uniaxial press. The compacted blends may be sintered in an inert atmosphere at a temperature in a range from about 650 °C to about 1000 °C. Silver may be infiltrated into the pores of the compacted and sintered structure to fill the pores with silver and to deposit silver on the first surface.

Alternately, a graded pore structure may be formed in the graded structure using different types and concentrations of binders during the compaction of the individual layer powders or blends. These binders during sintering evaporate and leave behind pores that can be later filled with the arcing surface material such as, for example, silver.

In one embodiment, the powder blends arranged in layered configuration may be subjected to HIP or spark plasma sintering to join the different layers together, thus making an integral contact tip 22.

### EXAMPLES

The following examples illustrate materials, methods, and results, in accordance with specific embodiments, and as such should not be construed as imposing limitations upon the claims. All components are commercially available from common suppliers.

The particle size and density details of some of the powders used are as given below in Table 1. Example compositions of some parts of the graded structure along with the base surface and arcing surface are as given in Table 2. One skilled in the art will appreciate that different particle sizes and particle densities may be used to formulate the graded structure. Further, the number of graded regions and the composition and structure of base surface, arcing surface, and graded regions may be varied as a result of routine experiments to form a further improved contact tip structure.

**Table 1.**

| Material | Size (microns) | Apparent Density (g/cc) |
|---|---|---|
| Silver | 6.0-9.0 | 1.7-2.2 |
| Tungsten | 4.5-5.5 | 2.9-3.7 |
| Tungsten Carbide | 1.5-7.0 | 4.0-4.7 |
| Nickel | 4.0-7.0 | 1.9-2.7 |
| Graphite | 40.0-45.0 | 1.9-2.2 |

**Table 2.**

| Base Surface | Example Compositions of Graded Contacts | Arcing Surface |
|---|---|---|
| 100% Cu | Ag (40-90wt %) - Ni (60-10 wt%) | 100% Ag |
| 100% Cu | Ag (15-50wt %) - WC (85-50wt %) | 100% Ag |
| 100% Cu | AgC (93-99 wt %) - C (7-1wt %) | 100% Ag |
| 100% Cu | Ag (15-50wt %) - W (85-50wt %) | 100% Ag |

Primarily three methods for the formation of the above-mentioned graded structure were explored. A press-sinter-repress (PSR) method was utilized using a uniaxial load of about 6-12 ton over a cross-sectional area of about 50-130 mm² to initially compact the base surface, graded structure, and arcing surface together. The compacted structure was sintered in a temperature range from about 650 °C to about 1000 °C for a time duration from about 10 minutes to about 60 minutes in an inert atmosphere of about 2-4% hydrogen in nitrogen or argon. The sintered structure was then further pressed with a pressure of about 36 to 60 ksi using cold iso-static pressing method.

In another method, spark plasma sintering (SPS) method was used to join the base surface and arcing surface using a graded structure. A pressure of about 30-50 MPa and an effective sintering temperature from about 650 °C to about 775 °C was used for a hold time of about 2- 10 minutes duration to compact the structure.

In a hot iso-static pressing (HIP) method, the starting powders and blends were subjected to a uniaxial load of about 6-12 tons over a cross-sectional area of about 50-130 mm² for initial pressing, and then further pressed at a temperature range from about 650 °C to about 750 °C at a pressure range from about 20 ksi to about 30 ksi for about 1- 3 hours' time duration.

## Claims

1. A system, comprising:
a contact tip (22) comprising
an arcing surface (26);
a base surface (24); and
a graded structure (40) between the arcing surface (26) and the base surface (24),
wherein the graded structure (40) comprises
a first region (50) comprising a first surface (52) proximate to the arcing surface (26);
a second region (60) comprising a second surface (62) proximate to the base surface (24); whereby
an intermediate region is (70) disposed between the first region (50) and the second region (60), wherein
a concentration of silver in the graded structure (40) decreases with a gradient from the first surface (52) to the second surface (62).

2. The system of claim 1, wherein the graded structure (40) comprises a continuously graded architecture between the first surface (52) and the second surface (62).

3. The system of claim 1 or claim 2, wherein a concentration of copper in the graded structure (40) decreases from the second surface (62) to the first surface (52).

4. The system of any preceding claim, wherein the arcing surface (26) comprises substantially 100% silver.

5. The system of any preceding claim, wherein the base surface (24) comprises substantially 100% copper.

6. The system of any preceding claim, wherein the graded structure (40) further comprises tungsten, tungsten carbide, molybdenum, nickel, carbon, or a combination of the foregoing.

7. The system of any preceding claim, wherein the graded structure (40) comprises a metal mixture.

8. The system of any preceding claim, wherein the metal mixture comprises a metal carbide, a silver-tungsten alloy, a silver-nickel alloy, silver tungsten carbide composite, silver molybdenum composite, or a combination of the foregoing.

9. The system of any preceding claim, wherein a concentration of the metal mixture in the intermediate region (70) is substantially higher than the concentration of the metal mixture at the second region (60).

10. The system of any preceding claim, wherein the graded structure (40) comprises a gradation in the composition of the metal mixture.

11. The system of any preceding claim, wherein the first region (50) comprises a silver-nickel metal mixture; the intermediate region (70) comprises a silver-copper-nickel metal mixture; and the second region (60) comprises substantially copper.

12. The system of any preceding claim, wherein the first region (50) comprises a silver-tungsten metal mixture; the intermediate region (70) comprises a silver-copper-tungsten metal mixture; and the second region (60) comprises substantially 100 wt% of copper.

13. The system of any preceding claim, wherein the first region (50) comprises a silver graphite metal mixture in the first region (50); the intermediate region (70) comprises a silver-copper carbide metal mixture; and the second region (60) comprises substantially 100 wt% copper.

14. The system of any preceding claim, wherein the first region (50) comprises a silver-tungsten carbide metal mixture in the first region (50); the intermediate region (70) comprises a copper-tungsten carbide-tungsten metal mixture; and the second region (60) comprises substantially 100 wt% copper.

15. A method of forming a contact tip (22) according to claim 1, comprising:
preparing starting materials for a first region (50), an intermediate region (70), and a second region (60) of the contact tip (22);
the first region (50) contains silver and the intermediate region (70) contains silver;
sequentially adding the starting materials of the first, intermediate, and second regions (50, 60, 70) to a container to form a graded blend of starting materials;
compacting and heat-treating the graded blend in the container to form the contact tip (22) comprising a graded structure (40), whereby
a concentration of silver in the graded structure (40) decreases from the first region (50) to the second region (60), wherein
the concentration of silver in the intermediate region (70) is less than the concentration of silver in the first region (50).

## Patentansprüche

1. System, umfassend:
eine Kontaktspitze (22) umfassend
eine Lichtbogenüberschlagsoberfläche (26);
eine Basisoberfläche (24); und
eine abgestufte Struktur (40) zwischen der Lichtbogenüberschlagsoberfläche (26) und der Basisoberfläche (24), wobei die abgestufte Struktur (40) Folgendes umfasst:
ein erstes Gebiet (50), das eine erste Oberfläche (52) umfasst, bei der Lichtbogenüberschlagsoberfläche (26);
ein zweites Gebiet (60), das eine zweite Oberfläche (62) umfasst, bei der Basisoberfläche (24);
ein Zwischengebiet (70) zwischen dem ersten Gebiet (50) und dem zweiten Gebiet (60) angeordnet, wobei
eine Konzentration von Silber in der abgestuften Struktur (40) mit einem Gradienten von der ersten Oberfläche (52) zu der zweiten Oberfläche (62) abnimmt.

2. System nach Anspruch 1, wobei die abgestufte Struktur (40) eine kontinuierlich abgestufte Architektur zwischen der ersten Oberfläche (52) und der zweiten Oberfläche (62) umfasst.

3. System nach Anspruch 1 oder 2, wobei eine Konzentration von Kupfer in der abgestuften Struktur (40) von der zweiten Oberfläche (62) zu der ersten Oberfläche (52) abnimmt.

4. System nach einem vorhergehenden Anspruch, wobei die Lichtbogenüberschlagsoberfläche (26) im Wesentlichen 100% Silber umfasst.

5. System nach einem vorhergehenden Anspruch, wobei die Basisoberfläche (24) im Wesentlichen 100% Kupfer umfasst.

6. System nach einem vorhergehenden Anspruch, wobei die abgestufte Struktur (40) weiterhin Wolfram, Wolframcarbid, Molybdän, Nickel, Kohlenstoff oder eine Kombination der vorausgegangenen umfasst.

7. System nach einem vorhergehenden Anspruch, wobei die abgestufte Struktur (40) eine Metallmischung umfasst.

8. System nach einem vorhergehenden Anspruch, wobei die Metallmischung ein Metallcarbid, eine Silber-Wolfram-Legierung, eine Silber-Nickel-Legierung, ein Silber-Wolfram-Carbid-Komposit, ein Silber-Molybdän-Komposit oder eine Kombination der vorausgegangenen umfasst.

9. System nach einem vorhergehenden Anspruch, wobei eine Konzentration der Metallmischung in dem Zwischengebiet (70) wesentlich höher ist als die Konzentration der Metallmischung beim zweiten Gebiet (60).

10. System nach einem vorhergehenden Anspruch, wobei die abgestufte Struktur (40) eine Abstufung in der Zusammensetzung der Metallmischung umfasst.

11. System nach einem vorhergehenden Anspruch, wobei das erste Gebiet (50) eine Silber-Nickel-Metallmischung umfasst; das Zwischengebiet (70) eine Silber-Kupfer-Nickel-Metallmischung umfasst und das zweite Gebiet (60) im Wesentlichen Kupfer umfasst.

12. System nach einem vorhergehenden Anspruch, wobei das erste Gebiet (50) eine Silber-Wolfram-Metallmischung umfasst; das Zwischengebiet (70) eine Silber-Kupfer-Wolfram-Metallmischung umfasst und das zweite Gebiet (60) im Wesentlichen 100 Gew.-% Kupfer umfasst.

13. System nach einem vorhergehenden Anspruch, wobei das erste Gebiet (50) eine Silber-Graphit-MetallMischung umfasst; das Zwischengebiet (70) eine Silber-Kupfercarbid-Metallmischung umfasst und das zweite Gebiet (60) im Wesentlichen 100 Gew.-% Kupfer umfasst.

14. System nach einem vorhergehenden Anspruch, wobei das erste Gebiet (50) eine Silber-Wolframcarbid-Metallmischung umfasst; das Zwischengebiet (70) eine Kupfer-Wolframcarbid-Wolfram-Metallmischung umfasst und das zweite Gebiet (60) im Wesentlichen 100 Gew.-% Kupfer umfasst.

15. Verfahren zum Ausbilden einer Kontaktspitze (22) nach Anspruch 1, umfassend:
Vorbereiten von Ausgangsmaterialien für ein erstes Gebiet (50), ein Zwischengebiet (70) und ein zweites Gebiet (60) der Kontaktspitze (22);
das erste Gebiet (50) enthält Silber und das Zwischengebiet (70) enthält Silber;
sequenzielles Hinzufügen der Ausgangsmaterialien des ersten, Zwischen- und zweiten Gebiets (50, 60, 70) in einen Behälter, um eine abgestufte Mischung von Ausgangsmaterialien auszubilden;
Verdichten und Wärmebehandeln der abgestuften Mischung in dem Behälter, um die eine abgestufte Struktur (40) umfassende Kontaktspitze (22) auszubilden,
eine Konzentration von Silber in der abgestuften Struktur (40) nimmt von dem ersten Gebiet (50) zu dem zweiten Gebiet (60) ab, wobei
die Konzentration von Silber im Zwischengebiet (70) unter der Konzentration von Silber im ersten Gebiet (50) liegt.

## Revendications

1. Système, comprenant :
une pointe de contact (22) comprenant une surface de formation d'arc (26) ;
une surface de base (24) ; et
une structure à gradient (40) entre la surface de formation d'arc (26) et la surface de base (24), la structure à gradient (40) comprenant
une première région (50) comprenant une première surface (52) proche de la surface de formation d'arc (26) ;
une deuxième région (60) comprenant une deuxième surface (62) proche de la surface de base (24) ; d'où il résulte que
une région intermédiaire (70) est disposée entre la première région (50) et la deuxième région (60), dans lequel
une concentration d'argent dans la structure à gradient (40) diminue avec un gradient de la première surface (52) à la deuxième surface (62).

2. Système de la revendication 1, dans lequel la structure à gradient (40) comprend une architecture à gradient continu entre la première surface (52) et la deuxième surface (62).

3. Système de la revendication 1 ou la revendication 2, dans lequel une concentration de cuivre dans la structure à gradient (40) diminue de la deuxième surface (62) à la première surface (52).

4. Système d'une quelconque revendication précédente, dans lequel la surface de formation d'arc (26) comprend sensiblement 100 % d'argent.

5. Système d'une quelconque revendication précédente, dans lequel la surface de base (24) comprend sensiblement 100 % de cuivre.

6. Système d'une quelconque revendication précédente, dans lequel la structure à gradient (40) comprend en outre du tungstène, du carbure de tungstène, du molybdène, du nickel, du carbone, ou une combinaison des éléments précédents.

7. Système d'une quelconque revendication précédente, dans lequel la structure à gradient (40) comprend un mélange métallique.

8. Système d'une quelconque revendication précédente, dans lequel le mélange métallique comprend un carbure métallique, un alliage argent-tungstène, un alliage argent-nickel, un composite argent-carbure de tungstène, un composite argent-molybdène, ou une combinaison des éléments précédents.

9. Système d'une quelconque revendication précédente, dans lequel une concentration du mélange métallique dans la région intermédiaire (70) est sensiblement supérieure à la concentration du mélange métallique au niveau de la deuxième région (60).

10. Système d'une quelconque revendication précédente, dans lequel la structure à gradient (40) présente une gradation dans la composition du mélange métallique.

11. Système d'une quelconque revendication précédente, dans lequel la première région (50) comprend un mélange métallique argent-nickel ; la région intermédiaire (70) comprend un mélange métallique argent-cuivre-nickel ; et la deuxième région (60) comprend en grande partie du cuivre.

12. Système d'une quelconque revendication précédente, dans lequel la première région (50) comprend un mélange métallique argent-tungstène ; la région intermédiaire (70) comprend un mélange métallique argent-cuivre-tungstène ; et la deuxième région (60) comprend sensiblement 100 % en poids de cuivre.

13. Système d'une quelconque revendication précédente, dans lequel la première région (50) comprend un mélange métallique argent-graphite; la région intermédiaire (70) comprend un mélange métallique argent-carbure de cuivre ; et la deuxième région (60) comprend sensiblement 100 % en poids de cuivre.

14. Système d'une quelconque revendication précédente, dans lequel la première région (50) comprend un mélange métallique argent-carbure de tungstène; la région intermédiaire (70) comprend un mélange métallique cuivre-carbure de tungstène-tungstène ; et la deuxième région (60) comprend sensiblement 100 % en poids de cuivre.

15. Procédé de formation d'une pointe de contact (22) selon la revendication 1, comprenant :
la préparation de matières premières pour une première région (50), une région intermédiaire (70) et une deuxième région (60) de la pointe de contact (22) ;
la première région (50) contient de l'argent et la région intermédiaire (70) contient de l'argent ;
l'ajout successif des matières premières de la première région, la région intermédiaire et la deuxième région (50, 60, 70) à un récipient pour former un mélange à gradient de matières premières ;
le compactage et le traitement thermique du mélange à gradient dans le récipient pour former la pointe de contact (22) comprenant une structure à gradient (40), d'où il résulte que
une concentration d'argent dans la structure à gradient (40) diminue de la première région (50) à la deuxième région (60), dans lequel
la concentration d'argent dans la région intermédiaire (70) est inférieure à la concentration d'argent dans la première région (50).
